

## UNITED STATES PATENT OFFICE

MAURICE E. BARKER, OF THE UNITED STATES ARMY, CAMBRIDGE, MASSACHUSETTS,  
ASSIGNOR OF ONE-FIFTH TO HARRY H. SEMMES, OF WASHINGTON, DISTRICT OF  
COLUMBIA

## ALLOY

No Drawing.

Application filed September 5, 1928. Serial No. 304,161.

(GRANTED UNDER THE ACT OF MARCH 3, 1883, AS AMENDED APRIL 30, 1928; 370 O. G. 757)

This invention described herein may be manufactured and used by or for the Government for government purposes, without the payment to me of any royalty thereon.

5 My invention relates to the art of metallurgy and more particularly to alloys containing silver together with other less expensive metals.

Silver is today one of the most widely used metals for ornamental, and other purposes, where a substantially inert metal is necessary. Although pure silver is substantially inert to ordinary materials and is not subject to corrosion, as are iron and steel, yet 10 its use in articles wherein durability and hardness are essential is not practical. Many attempts have been made to avoid this undesirable property, such as by silverplating metals like iron and steel, and alloying silver 15 with other metals.

Silver is also a relatively expensive metal, and in many instances its use has been restricted because of its cost.

Silverplating, although employed to a 25 large extent, is not entirely satisfactory as in the course of time, especially if the article is subjected to much wear or erosion, the coating of silver plate will vanish, leaving the metal of which the article is formed exposed.

30 Articles from which the silver plate is worn are, besides being unsightly, subject to corrosion to the same extent as if they had never been plated.

The alloys heretofore perfected have not 35 been entirely satisfactory as they have been costly, and have not had the properties desired to meet the conditions which such substances should be capable of withstanding.

Nickel has in many instances been substituted for silver but despite its hard and durable properties, it has not been successfully employed because it lacks the attractiveness and inertness of silver.

An object of this invention is to produce 45 a substitute for metallic silver having as many of the desirable properties of silver and as few of the undesirable properties of silver as is possible.

Another object of my invention is to produce 50 alloys of silver having the inert and or-

namental properties of silver together with the durable characteristics of other metals.

Still another object of my invention is to produce a durable silver-like metal suitable for use in constructing articles for the household such as cutlery and other ware and as a general substitute for silver. 55

With these and other objects in view, the invention consists in the process and product herein set forth, with the understanding that 60 the several necessary elements entering into the composition of the alloys may be varied in proportion, without departing from the nature or scope of the invention.

It is particularly desirable in the manufacture of metallic articles, such as cutlery, tableware or other metallic products which may possibly be subjected to the corrosive effects of food, that some metal be available that will resist corrosion and yet will be durable and capable of undergoing changes in physical shape without detrimentally affecting the physical or chemical structure of the material. Also, the metal of which cutlery 65 is made should be somewhat hard so as to be 70 capable of holding a sharp cutting edge. 75

My invention contemplates the production of alloys containing relatively small amounts of silver which have some properties similar to silver and which are especially desirable for use in the manufacture of tableware and other articles that must be durable and yet resist corrosion. 80

The alloys constituting this invention contain nickel, iron and silver in amounts requisite for producing alloys having the properties desired. 85

Any of the standard methods for preparing alloys may be employed in the production of the metal constituting my invention. 90 One particular method is to form alloys of one metal with each of the others and then fuse the two preliminary alloys into the final product. Such a procedure or a similar one is essential as it is absolutely necessary that all of the metals entering into the alloy be completely fused and thoroughly dissolved in each other. 95

If the metals entering into the alloy are 100 not completely fused and the solution formed

is not homogeneous, the resulting mixture will not exhibit the properties of a properly made alloy containing the same ingredients.

It is also essential in the production of alloys according to my invention, that the materials used in the preparation thereof be of substantial purity. The highest purity of commercial grade of the metals should be used in preparing these alloys to produce a satisfactory substitute for silver. High purity of the iron used in preparing silver substitutes is very essential to produce alloys having the properties desired. Of course silver substitutes for certain purposes not so exacting in requirements can be prepared from less pure metals.

Although the composition of the alloy constituting my invention may be varied within rather wide limits without sacrificing any of the desirable properties, it is preferable to form the silver substitute alloy of a composition within the limits given below.

|        |            |
|--------|------------|
| Iron   | 45% to 55% |
| Nickel | 37% to 47% |
| Silver | 3% to 13%  |

With such a range of possible variations in the composition of the alloys, the latter can be manufactured to meet all demands of the trade, from relatively cheap silver substitutes to more expensive ones. Thus many articles heretofore made of metals lacking the desirable non-corrosive and ornamental properties of silver can now be economically and efficiently made from my alloy.

An alloy included within the range of variations of components of the composition given above and having the most desirable and the least undesirable properties is represented by the following composition.

|        |     |
|--------|-----|
| Iron   | 50% |
| Nickel | 42% |
| Silver | 8%  |

This alloy containing only 8% of silver is a very valuable substitute for silver, in that it can be fairly cheaply produced and yet sufficiently meets all demands of resistance to corrosion and beauty for which silver is used, together with the durability of iron and other similar metals. One essential property of a metal entering into the manufacture of variously shaped articles is that of ease of working. This particular property is characteristic of my alloy, thus making it also desirable from the actual construction point of view.

Thus my invention accomplishes the production of alloys having all the desirable qualities of silver for ornamental use and at the same time possessing greater tensile strength, ease of working, and resistance to corrosion in the ordinary air and in contact with ordinary foods. These alloys can be

used especially for the production of cutlery, flat pieces and other articles used on the table, though of course there are other uses to which they can be put. Alloys such as described do not require silver plating in order to present all the pleasing appearance of sterling silver, but enable articles of solid ware of silver appearance to be made at a price which can compete most favorably with the best of plated ware.

As the composition can be varied within a wide range it is possible to produce a variety of alloys suitable to meet all demands of the trade, depending on the use to which the material is to be subjected.

Although I have described a preferred embodiment of my invention, that is alloys of definite composition, I wish it to be understood that the composition of the alloys may be varied within rather wide limits and yet be within the scope of my invention.

I claim:

1. An alloy containing 37% to 47% nickel, 45% to 55% iron and 3% to 13% silver.
2. An alloy containing 50% iron, 42% nickel and 8% silver.
3. An alloy containing 39 to 45% nickel, 47 to 53% iron and 5 to 11% silver.
4. An alloy containing 40 to 44% nickel, 48 to 52% iron, and 6 to 10% silver.

In testimony whereof I affix my signature.

MAURICE E. BARKER.

100

105

110

115

120

125

130